

[54] **SOLUTION CAST DOUBLE BASE PROPELLANTS AND METHOD**

[75] Inventor: **Donald E. Elrick**, Rawlings, Md.

[73] Assignee: **The United States of America as represented by the Secretary of the Navy**, Washington, D.C.

[22] Filed: **Jan. 30, 1964**

[21] Appl. No.: **341,459**

[52] U.S. Cl. .... **149/2**; 149/92; 149/95; 149/98; 264/3 R; 264/3 C

[51] Int. Cl. <sup>2</sup> .... **C06B 45/00**

[58] Field of Search .... 149/96, 97, 98, 99, 18, 149/19, 2, 95, 92; 264/3 R, 3 C

[56] **References Cited**

UNITED STATES PATENTS

|           |         |              |        |
|-----------|---------|--------------|--------|
| 2,916,778 | 12/1959 | O'Neill..... | 149/96 |
| 2,967,098 | 1/1961  | Weil.....    | 149/19 |
| 3,002,830 | 10/1961 | Barr.....    | 149/19 |
| 3,033,715 | 5/1962  | Preckel..... | 149/96 |
| 3,036,939 | 5/1962  | Camp.....    | 149/19 |

3,106,498 10/1963 Grable ..... 149/96

Primary Examiner—Stephen J. Lechert, Jr.  
Attorney, Agent, or Firm—R. S. Sciascia; Roy Miller

**EXEMPLARY CLAIM**

1. A method for the preparation of a double base propellant grain which comprises the steps of

1. pretreating nitrocellulose by
  - a. stirring 100 grams of dry nitrocellulose into a solution of 2 grams of phenyl isocyanate in 500 grams of carbon tetrachloride,
  - b. filtering the resulting mixture and
  - c. drying the residue;
2. rotationally stirring 15 parts by weight of the pretreated nitrocellulose with 3 parts red lead, 1 part nitrodiphenylamine, 57.1 parts by weight nitroglycerin and 23.6 parts by weight triacetin until a viscous mixture results,
3. adding to this mixture tolylene diisocyanate,
4. transferring the resulting mixture under reduced pressure to a container and,
5. curing for 5 days at 50° C.

**9 Claims, No Drawings**

## SOLUTION CAST DOUBLE BASE PROPELLANTS AND METHOD

This invention relates to high performance solution cast double base propellant compositions and to the method of preparation.

Propellant systems containing nitrocellulose, nitroglycerin and other ingredients have been prepared in a number of ways. Cast propellants are generally prepared by first preparing small, hard, high density casting powder particles containing colloided nitrocellulose and other additives and then casting and curing in a suitable container. Other cast propellants are prepared using a plastisol process in which very small particles containing colloided nitrocellulose are mixed with various additives and a casting solvent until a desired viscosity is attained in the mixture is then cast. Extruded propellants require mixing of the necessary ingredients and extruding under high pressure with tremendous pressures being required for larger grains. The present invention relates generally to improvements in preparing propellant systems and more particularly to new and improved solution cast propellants which require no colloided nitrocellulose particles and only mixing and casting containers are needed.

The primary object of the present invention is a means of preparing high performance propellants which can be liquid loaded into a motor and by means of crosslinking converted to a solid grain bonded to the rocket motor.

Another object is the provision of an improved casting system which offers the economic advantages of reduced time, equipment, and labor.

A further object is to provide a method whereby 35 grains of intricate geometry can be readily cast.

Other objects and many of the attendant advantages of this invention will be readily appreciated as the same become better understood in the following detailed description.

This invention involves the preparation of high performance propellants by dissolving lacquer grade nitrocellulose in nitroglycerin or in a casting solvent and crosslinking the nitrocellulose by use of a polyisocyanate to form upon curing a relatively tough gel. A lead salt, which serves as a crosslinking catalyst and a ballistic modifier, is incorporated into the solution. By varying the ballistic modifier and the heat of explosion of the matrix, compositions of varying burning rates can be prepared. These mixtures can be liquid loaded into rocket motors to produce case bonded propellants. The method involved herein is concerned with (1) the solution of a lacquer grade nitrocellulose in an explosive solvent, (2) the use of any polyisocyanate as a crosslinking agent, (3) the ballistic modification of the composition by any modifier, which does not adversely affect the reaction of nitrocellulose with an isocyanate. If the ballistic modifier should not be a catalyst for the urethane crosslink formation, such a catalyst may be added to the composition. If the modifier should have an adverse effect upon urethane formation, the modifier may be coated to prevent this adverse effect and a crosslinking catalyst may be added to the composition.

Other crosslinking systems can be used, including titanates, epoxides, anhydrides, etc.

A more comprehensive understanding of this invention is obtained by reference to the following example:

### EXAMPLE I

10 parts dry (11.9%N) nitrocellulose  
3 parts red lead  
1 part ethyl Centralite  
60.1 parts nitroglycerin  
24.9 parts triacetin

were rotationally stirred until nitrocellulose had been 10 dissolved. To the viscous mixture was added 1.2 parts of tolylene diisocyanate and the mixture was transferred under pressure to a steel motor. This mixture, which weight 470 g. and had a heat of explosion of 804 cal./g., was allowed to cure for about 56 days at about 15 25°C. to produce a case bonded propellant with the appearance of a gel. The propellant was fired at a K of 1038 to obtain the following data:

|                                 |                |
|---------------------------------|----------------|
| Burning time                    | 26.9 sec.      |
| Burning rate                    | 0.093 in./sec. |
| Average pressure during burning | 525 psi.       |

### EXAMPLE II

25 The nitrocellulose used in this example was first pre-treated. Dry nitrocellulose (100 grams) was stirred with a solution of 2 grams of phenylisocyanate in 500 grams of carbon tetrachloride, filtered, and dried. Then,

15 parts pretreated nitrocellulose  
3 parts red lead  
1 part 2-nitrodiphenylamine  
57.1 parts nitroglycerin  
23.6 parts triacetin

were rotationally stirred until nitrocellulose had been dissolved to form a viscous mixture. To this mixture 0.4 parts of tolylene diisocyanate was added. The mixture was then transferred under reduced pressure to a steel 40 motor coated internally with a 1 mil binder of partially crosslinked cellulose acetate. The mixture which weighed 950 grams and had a heat of explosion of 824 cal./gram, was allowed to cure for 5 days at 50°C. to produce a case bonded propellant with the characteristics of a relatively tough gel. The propellant was fired at a K of 793 to obtain the following data:

|                                 |                |
|---------------------------------|----------------|
| Burning time                    | 58.4 sec.      |
| Burning rate                    | 0.086 in./sec. |
| Average pressure during burning | 370 psi        |

### EXAMPLE III

55 15 parts pretreated nitrocellulose (see Example II)  
3 parts lead stearate  
2 parts nitrodiphenylamine  
56.8 parts nitroglycerin  
22.7 parts triacetin

were rotationally stirred until nitrocellulose was in solution forming a viscous mixture to which 0.6 parts of tolylene diisocyanate was added. The mixture was then transferred under reduced pressure to a steel motor, coated internally with 1 mil binder of partially cross-linked cellulose acetate. The mixture which weighed 60 925 grams and had a heat of explosion of 748 cal./g. was allowed to cure for 7 days at 50°C. to produce a case bonded propellant with the characteristics of a rel-

atively tough gel. The propellant was fired at a K of 903 to obtain the following data:

|                                 |                |
|---------------------------------|----------------|
| Burning time                    | 38.2 sec.      |
| Burning rate                    | 0.131 in./sec. |
| Average pressure during burning | 740 psi.       |

#### EXAMPLE IV

|                                                    |  |
|----------------------------------------------------|--|
| 20 parts by weight of casting powder consisting of |  |
| 75% (11.9%N, 20 cp.) nitrocellulose                |  |
| 23% nitroglycerin                                  |  |
| 2% nitrodiphenylamine                              |  |
| 3 parts dibasic lead phthalate                     |  |
| 1.9 parts triacetin                                |  |
| 75.1 parts casting solvent containing              |  |
| 70% nitroglycerin                                  |  |
| 29% triacetin                                      |  |
| 1% nitrodiphenylamine                              |  |

were rotationally stirred until a viscous mixture formed. To this mixture 0.3 parts phenyl isocyanate were added and the mixture again rotationally stirred. Any unreacted isocyanate was removed under reduced pressure. Then 0.4 parts of tolylene diisocyanate was added to the mixture which was poured into a steel motor, coated internally with a 1 mil binder of partially crosslinked cellulose acetate. The mixture was allowed to cure for 3 days at about 50°C. to produce a case bonded propellant with characteristics of a tough gel. The propellant was fired at a K of 903 to obtain a burning rate of 0.33 at a pressure of 2160 psi.

#### EXAMPLE V

|                                                |  |
|------------------------------------------------|--|
| 22.2 parts by weight casting powder containing |  |
| 70% (11.9%N, 20 cp.) nitrocellulose            |  |
| 13.6% nitroglycerin                            |  |
| 14% dibasic lead phthalate                     |  |
| 1.4% nitrodiphenylamine                        |  |
| 77.8 parts of a casting solvent containing     |  |
| 75% nitroglycerin                              |  |
| 24% triacetin                                  |  |
| 1% nitrodiphenylamine                          |  |

were rotationally stirred until the nitrocellulose was in solution forming a viscous mixture. After 0.3 parts of phenyl isocyanate had been added, the viscous mixture was rotationally stirred and excess isocyanate was removed under reduced pressure. Then 0.4 parts tolylene diisocyanate was added and the mixture transferred to a steel motor, coated internally with a 1 mil binder of partially crosslinked cellulose acetate. The mixture, which had a heat of explosion of 953 cal./g., was allowed to cure for three days at 50°C. to produce a case bonded propellant. A total of three motors were prepared in the above manner to obtain the following ballistic data: a rate of 0.39 in./sec. at 1000 psi with a slope of 0.20 from 500-1000 psi. A cast dumbbell specimen gave the following data: at -20°F. maximum stress 44 psi, modulus 49 psi and elongation greater than 91%; at -40°F. maximum stress 67 psi, modulus 233 psi and elongation 93%.

#### EXAMPLE VI

|                                      |  |
|--------------------------------------|--|
| 17.9 parts casting powder containing |  |
| 70% (11.9%N, 20 cp.) nitrocellulose  |  |
| 13.6% nitroglycerin                  |  |
| 14% dibasic lead phthalate           |  |
| 1.4% carbon black                    |  |

|                                       |  |
|---------------------------------------|--|
| 1% nitrodiphenylamine                 |  |
| 82.1 parts casting solvent containing |  |
| 97% diglycol dinitrate                |  |

3% nitrodiphenylamine

were rotationally stirred until the nitrocellulose was in solution forming a viscous mixture. After 0.3 parts phenyl isocyanate had been added, the viscous mixture was rotationally stirred at 35°C. for two hours and excess isocyanate was removed under reduced pressure. To the mixture was added 0.4 parts of tolylene diisocyanate and the mixture was transferred at 35°C. under reduced pressure to steel motors, coated internally with 1 mil crosslinked cellulose acetate binder. The mixture which had a heat of explosion of 865 cal./gram was allowed to cure for three days at 50°C. to produce case bonded propellants having the characteristics of relatively tough gel. There was obtained at a K of 386 a burning rate of 0.48 in./sec. at 1365 psi, and at a K of 244 a burning rate of 0.44 in./sec. at 675 psi.

#### EXAMPLE VII

|                                       |  |
|---------------------------------------|--|
| 22.2 parts casting powder containing  |  |
| 70% nitrocellulose (11.9%N)           |  |
| 13.6% nitroglycerin                   |  |
| 14% dibasic lead phthalate            |  |
| 1.4% carbon black                     |  |
| 1% nitrodiphenylamine                 |  |
| 77.8 parts casting solvent containing |  |
| 75% glycol dinitrate                  |  |
| 24% triacetin                         |  |
| 1% nitrodiphenylamine                 |  |

were rotationally stirred until the nitrocellulose was in solution. After 0.25 parts of phenyl isocyanate had been added, the viscous mixture was again rotationally stirred and excess isocyanate was removed under reduced pressure. To the mixture was added 0.4 parts of tolylene diisocyanate and the mixture was transferred under reduced pressure to a steel motor, coated internally with a binder of partially crosslinked cellulose acetate. The mixture which had a heat of explosion of 937 cal./gram was allowed to cure for three days at 50°C. to produce a tough gel. The case bonded propellant was fired at a K of 396 to obtain a burning rate of 0.34 in./sec. at 865 psi.

#### EXAMPLE VIII

|                                       |  |
|---------------------------------------|--|
| 22.2 parts casting powder containing  |  |
| 70% nitrocellulose (11.9%N)           |  |
| 22.9% nitroglycerin                   |  |
| 4.7% tribasic lead maleate            |  |
| 1% nitrodiphenylamine                 |  |
| 1.4% carbon black                     |  |
| 77.8 parts casting solvent containing |  |
| 75% nitroglycerin                     |  |
| 24% triacetin                         |  |
| 1% nitrodiphenylamine                 |  |

were rotationally stirred until viscous mixture resulted to which 0.25 parts phenyl isocyanate were added. The mixture was stirred for two days and excess isocyanate was removed under reduced pressure. Tolylene diisocyanate (0.4 parts) was added to the mixture which was transferred under pressure to two steel motors coated inside with a binder of partially crosslinked cellulose acetate. The mixture which had a heat of explosion of

989 cal./gram was allowed to cure at 50°C. to produce a soft gel of a case bonded propellant. The propellant was fired to obtain the following ballistic data: a rate of 0.34 in./sec. at 1000 psi with a slope of 0.57 from 500 – 1100 psi.

#### EXAMPLE IX

A slurry containing

27.4 parts by weight of 95% ethanol and  
72.6 parts by weight of mixture consisting of  
90.8% (12.2%N, 20 cp.) nitrocellulose  
6.1% tribasic lead maleate  
1.3% nitrodiphenylamine  
1.8% carbon black (Carbolac I)

was prepared and stirred for one hour in a Sigma Blade Mixer.

20.4 parts of the mixture

4.6 parts 95% ethanol  
75.0 parts of a casting solvent containing  
76.5% nitroglycerin  
22.6% triacetin  
0.9% nitrodiphenylamine

were rotationally stirred until a slightly viscous mixture formed. The ethanol was removed under reduced pressure and 0.25 parts of phenyl isocyanate was added. This mixture was rotationally stirred for one hour and excess isocyanate was removed under reduced pressure. To this mixture was added a total of 1.4 parts tolylene diisocyanate and the mixture was transferred under reduced pressure to a steel motor coated internally with a binder of partially crosslinked cellulose acetate. The mixture which had a heat of explosion of 989 cal./gram was cured for three days at 50°C. to produce a soft gel of case bonded propellant. The propellant was fired at a K of 178 to obtain a burning rate of 0.28 in./sec. at 650 psi.

#### EXAMPLE X

To a mixture of 4.5 grams of nitrocellulose (11.9%N), 0.9 grams of dibasic lead phthalate, 0.06 grams of nitrodiphenylamine and 0.09 grams of carbon black (Carbolac I) in a large amount of methylene chloride was added with stirring a total of 27.6 grams of 99% nitroglycerin — 1% ethyl Centralite and 0.08 grams of phenyl isocyanate. After methylene chloride and excess isocyanate were removed, 0.12 grams of tolylene diisocyanate was added and the mixture was placed in strand molds, cured for two days at 50°C. and fired to obtain burning rates of 0.73 and 0.82 in./sec. at 810 and 1010 psi respectively.

#### EXAMPLE XI

A solution containing 20 parts dry nitrocellulose (11.9%N) and 80 parts dimethylsulfoxide was poured through a perforated plate and allowed to fall freely for 16 inches through air into water. The resulting pellets were extracted with water and dried to obtain porous nitrocellulose pellets with a loading density of 0.2 g./ml.

13.6 parts of these porous pellets  
83.2 parts of a casting solvent containing  
99% nitroglycerin  
1% ethyl Centralite  
2.7 parts dibasic lead phthalate  
0.3 parts carbon black (Carbolac I)

0.2 parts nitrodiphenylamine

were mixed by rotational stirring and evacuation under reduced pressure until a viscous mixture resulted.

5 About 0.25 parts phenyl isocyanate was then added and stirred. Excess isocyanate was removed under reduced pressure then 0.3 parts of tolylene diisocyanate was added and the mixture was cast in strand molds and in a steel rocket motor lined with partially crosslinked 10 cellulose acetate. This propellant which had a heat of explosion of 1547 cal./gram was allowed to cure for three days at 50°C. and produced a relatively tough gel. Strand burning rates gave a burning rate of 1.14 in./sec. at 1000 psi with a slope of 0.56. The case bonded propellant in the motor was fired at a K of 81 to obtain a rate of 0.75 in./sec. at 500 psi.

#### EXAMPLE XII

To a stirred mixture of

20 1 part dibasic lead phthalate  
0.4 parts of nitrodiphenylamine in  
22.1 parts of triacetin at -40°C.,  
15 parts dry phenyl isocyanate pre-treated nitrocellulose was added with continuous stirring then  
61.5 parts of a casting solvent containing  
75% nitroglycerin  
24% triacetin  
1% nitrodiphenylamine

30 was added and the mixture was rotationally stirred until a slightly viscous slurry was formed. To this mixture a total of 1.6 parts of tolylene diisocyanate was added and the mixture transferred under reduced pressure to a steel rocket motor which had been coated with a partially crosslinked cellulose acetate. The mixture which had a heat of explosion of 412 cal./g., was allowed to cure for three days at 50°C. to produce a case bonded propellant with the characteristics of a slightly soft gel.

40 As described in the examples herein set out, this invention is concerned with the manufacture of high performance solution cast propellants which are prepared by first dissolving a lacquer grade nitrocellulose in nitroglycerin or casting solvent with the simultaneous solution or suspension of additives and then after addition of a polyisocyanate, pouring the mixture into a motor and curing.

45 Dissolution of the nitrocellulose is accomplished in a number of ways. Powder dry nitrocellulose which has been adequately wetted with casting solvent gradually dissolves to form a clear solution. Thorough wetting of nitrocellulose fibers is not easily accomplished in this manner; agglomerates of partially gelled nitrocellulose tend to form and may require long times to dissolve completely (Examples I, II and III). Quicker solution was obtained by slurring the nitrocellulose in cold triacetin and then adding the casting solvent. Dissolution of nitrocellulose is essentially negligible in the cold solvent and no agglomerates normally form. The dispersed nitrocellulose then dissolves rapidly when heated with stirring (Example XII). Other methods of obtaining the slurring state involve the use of non solvents. Nitrocellulose can be slurried in ethanol or methylene chloride and casting solvent added. The

55 slurring state is maintained as nitrocellulose is gradually dissolved during removal of the non-solvent. Ethanol is, however, not entirely satisfactory as lacquer grade nitrocellulose is slightly soluble therein (Example

IX). Methylene chloride is an excellent slurring medium and dissolution occurs rapidly. Methylene chloride wet nitrocellulose could satisfy the requirements of desensitized nitrocellulose (Example X). Other slurring media such as diethyl ether or chloroform should also be satisfactory. Much of the work has been done using a casting powder as the source of the nitrocellulose (Example IV to VIII). Optimum ballistic performance for a composition is obtained only if the modifiers are well dispersed. Casting powder was used herein as a source of the nitrocellulose to insure satisfactory modifier dispersion and optimum ballistic performance. Ballistic modifiers may also be dispersed in water wet nitrocellulose by subjecting such a mixture to the action of a sigma blade mixer. Incorporation of the modifiers in all solution cast propellants may be easily accomplished by premixing modifier and nitrocellulose. Another method for obtaining nitrocellulose solutions involves the use of porous nitrocellulose pellets. The casting solvent would rapidly wet the porous pellets allowing dissolution to occur rapidly. Good means of stirring would be required since the casting solvent wet powder tends to coalesce (Example XI).

Compositions containing this lacquer grade nitrocellulose had a tendency to gas upon curing an at elevated temperature (50°C.). Gassing did not occur upon curing at 25°C. (Example I). Gassing at elevated temperatures was eliminated by either treating anhydrous nitrocellulose with a dilute solution of phenyl isocyanate in carbon tetrachloride (Examples II, III, XII) or by adding phenyl isocyanate to the nitrocellulose casting solvent solution prior to final casting (Examples IV - XI). The reason for gassing is not known, though carbon dioxide can be formed when an isocyanate reacts with water or an acid. It appears that the gas formation with untreated nitrocellulose may be traceable to residual sulfate or the relatively high carboxyl content of the low molecular weight material. Moisture might be retained by this unusually high hygroscopic substance, this property also being characteristic of low molecular weight and the associated high concentration of end groups.

Although tolylene diisocyanate has been used in this work, other polyisocyanates can be used to obtain crosslinked products. The rate of reaction of hexamethylene diisocyanate or bitolylene diisocyanate with nitrocellulose is comparable to that of tolylene diisocyanate. The latter diisocyanate, which is a solid, would have to be added to the mixture in solution with a portion of the casting solvent. Other polyisocyanates such as polyaryl polyisocyanate or 3,3' dimethyl diphenylmethane 4,4 diisocyanate could also be substituted for tolylene diisocyanate. Other crosslinking systems can be used, including titanates, epoxides, anhydrides, etc.

The lead salt has a dual function of ballistic modifier and crosslinking catalyst. Red lead ( $Pb_3O_4$ ) has been used as a crosslinking catalyst (Examples I and II), since its catalysis of the nitrocellulose-isocyanate reaction would give the desired rate of crosslinking. About 60% of the isocyanate reacted in 20 hours and 80% in 40 hours at 55°C. The mixture containing the polyisocyanate must have sufficient pot life for a casting period of about three hours. Lead stearate was also a satisfactory catalyst (Example III) in that eight hours were required to react 60% of the isocyanate at 55°C. Dibasic lead phthalate (Examples IV to VII; X to XII) and tribasic lead maleate (Examples VIII and IX) have cat-

alytic effects similar to red lead although no rates have been determined. Compositions containing 3% red lead or lead stearate and having a heat of explosion of 750 - 825 cal./g. gave burning rate slopes of about 1 (Examples I to III). When the ballistic modifiers were 1% tribasic lead maleate and 0.3% carbon black and the heat of explosion of 989 cal./g. a

Other nitrocellulose of varying viscosity and nitrogen content have been incorporated in solution cast propellants and evaluated. The mixture that is poured into a rocket motor must be sufficiently viscous to prevent settling of solids such as ballistic modifiers and yet must be sufficiently fluid for pouring purposes. The strength of the resulting gel is dependent on the amount of nitrocellulose in the mixture. Thus the nitrocellulose that is best suited for solution cast propellants is the one processable at the highest attainable concentration in the mixture. The maximum workable concentration of various nitrocelluloses in solution cast propellants is as follows: for 12.6%N, 10 to 18 sec., military grade - 2.8% for 12.2%N, 5 to 6 sec. - 6.0%; for 11.0%, 1.4 sec. - 7% and for 11.9 to 12.2%N, 20 cp. - 15%. burning rate of 0.34 in./sec. at 1000 psi, and a slope of 0.57 was obtained (Example VIII). When 3% dibasic lead phthalate and 0.3% carbon black were the ballistic modifiers and the heat of explosion was 953 cal./g., a rate of 0.39 in./sec. at 1000 psi with a slope of 0.20 from 500 - 1000 psi was obtained (Example V). When 3% dibasic lead phthalate and 0.3% carbon black were the ballistic modifiers and the heat of explosion was 1547 cal./g., a rate of 1.14 in./sec. at 1000 psi with a slope of 0.56 from 500 - 1100 psi was obtained (Example XI).

Explosive plasticizers other than nitroglycerin have been incorporated into these propellants. When glycol dinitrate replaced most of the nitroglycerin in a composition containing 3% dibasic lead phthalate and 0.3% carbon black and having a heat of explosion of 937 cal./g., a burning rate of 0.34 in./sec. at 856 psi was obtained (Example VII). When diglycol dinitrate was used in a similar composition which had a heat of explosion of 865 cal./g., an interpolated burning rate of 0.46 in./sec. at 1000 psi was obtained (Example VI).

Other nitrocelluloses of varying viscosity and nitrogen content have been incorporated into solution cast propellants and evaluated. The mixture that is poured into a rocket motor must be sufficiently viscous to prevent settling of solids such as ballistic modifiers and yet must be sufficiently fluid for pouring purposes. The strength of the resulting gel is dependent on the amount of nitrocellulose in the mixture. Thus the nitrocellulose that is best suited for solution cast propellants is the one processable at the highest attainable concentration in the mixture. The maximum workable concentration of various nitrocelluloses in solution cast propellants is as follows: for 12.6%N, 10 to 18 sec., military grade - 2.8%; for 12.2%N, 5 to 6 sec. - 6.0%; for 11.0%, 1.4 sec. - 7% and for 11.9 to 12.2%N, 20 cp. - 15%.

Obviously many modifications and variations of the present invention are possible in the light of the above teachings. It is therefore to be understood that within the scope of the appended claims the invention may be practiced otherwise than as specifically described.

What is claimed is:

1. A method for the preparation of a double base propellant grain which comprises the steps of
  1. pretreating nitrocellulose by

- a. stirring 100 grams of dry nitrocellulose into a solution of 2 grams of phenyl isocyanate in 500 grams of carbon tetrachloride,
- b. filtering the resulting mixture and
- c. drying the residue;
2. rotationally stirring 15 parts by weight of the pre-treated nitrocellulose with 3 parts red lead, 1 part nitrodiphenylamine, 57.1 parts by weight nitroglycerin and 23.6 parts by weight triacetin until a viscous mixture results,
3. adding to this mixture tolylene diisocyanate,
4. transferring the resulting mixture under reduced pressure to a container and,
5. curing for 5 days at 50°C.

2. A method for the preparation of a double base propellant grain which comprises the steps of

1. stirring 22.2 parts by weight of a casting powder consisting of
  - a. 70% nitrocellulose
  - b. 13.6% nitroglycerin
  - c. 14% dibasic lead phthalate
  - d. 1.4% carbon black
  - e. 1% nitrodiphenylamine

with 77.8 parts by weight of a casting solvent consisting of

- a. 75% nitroglycerin
- b. 24% triacetin
- c. 1% nitrodiphenylamine

until a viscous mixture results,

2. adding while stirring 0.3 parts by weight phenyl isocyanate,

3. removing excess phenyl isocyanate under reduced pressure,

4. adding 0.4 parts by weight tolylene diisocyanate,

5. transferring the resulting mixture to a container and

6. curing for three days at 50°C.,

all percentages being by weight.

3. A method for the preparation of a propellant grain which comprises the steps of

1. providing porous nitrocellulose pellets prepared by
  - a. mixing 20 parts by weight dry nitrocellulose with 80 parts by weight dimethylsulfoxide to form a solution,
  - b. pouring said solution through a perforated plate through air into water to form pellets,
  - c. extracting said pellets with water and
  - d. drying to obtain porous nitrocellulose pellets;
2. stirring

- 13.6 parts by weight of said pellets with 83.2 parts by weight of a casting solvent consisting of
  - a. 99% nitroglycerin and
  - b. 1% ethyl Centralite

2.7 parts by weight dibasic lead phthalate

0.3 parts by weight carbon black

0.2 parts by weight nitrodiphenylamine

until a viscous mixture results, while stirring

3. adding while stirring 0.25 parts phenyl isocyanate,
4. removing under reduced pressure excess isocyanate

5. adding 0.3 parts tolylene diisocyanate,

6. pouring the resulting mixture into a rocket motor, and

7. curing for three days at 50°C.

4. A propellant composition consisting essentially of

|   | Ingredients           | Parts by weight |
|---|-----------------------|-----------------|
| 5 | Nitrocellulose        | 10              |
|   | Red lead              | 3               |
|   | Ethyl Centralite      | 1               |
|   | Nitroglycerin         | 60.1            |
|   | Triacetin             | 24.9            |
|   | Tolylene diisocyanate | 1               |

5. A propellant composition consisting essentially of

|    | Ingredients                                                                         | Parts by weight |
|----|-------------------------------------------------------------------------------------|-----------------|
| 15 | Nitrocellulose degassed in a solution of phenyl isocyanate and carbon tetrachloride | 15              |
|    | Red lead                                                                            | 3               |
|    | Nitrodiphenylamine                                                                  | 1               |
|    | Nitroglycerin                                                                       | 57.0            |
|    | Triacetin                                                                           | 23.6            |
| 20 | Tolylene diisocyanate                                                               | 0.4.            |

6. A propellant composition consisting essentially of

|    | Ingredients                                                             | Parts by weight |
|----|-------------------------------------------------------------------------|-----------------|
| 25 | Nitrocellulose pellets                                                  | 13.6            |
|    | Casting solvent consisting of 99% nitroglycerin and 1% ethyl Centralite | 83.2            |
|    | Dibasic lead phthalate                                                  | 2.7             |
|    | Carbon black                                                            | 0.3             |
|    | Nitrodiphenylamine                                                      | 0.2             |
|    | Tolylene diisocyanate                                                   | 0.3.            |

7. A propellant composition consisting essentially of

|    | Ingredients                                                                                  | Parts by weight |
|----|----------------------------------------------------------------------------------------------|-----------------|
| 40 | Casting powder consisting of 75% nitrocellulose, 23% nitroglycerin and 2% nitrodiphenylamine | 20              |
|    | Dibasic lead phthalate                                                                       | 3               |
|    | Triacetin                                                                                    | 1.9             |
|    | Casting solvent consisting of 70% nitroglycerin, 29% triacetin and 1% nitrodiphenylamine     | 75.1            |
| 45 | Tolylene diisocyanate                                                                        | 0.4.            |

8. A propellant composition consisting essentially of

|    | Ingredients                                                                                                                                   | Parts by weight |
|----|-----------------------------------------------------------------------------------------------------------------------------------------------|-----------------|
| 55 | Casting powder consisting of 70% nitrocellulose, 13.6% nitroglycerin, 14% dibasic lead phthalate, 1.4% carbon black and 1% nitrodiphenylamine | 17.9            |
|    | Casting solvent consisting of 97% diglycol dinitrate and 3% nitrodiphenylamine                                                                | 82.1            |
|    | Tolylene diisocyanate                                                                                                                         | 0.4.            |

9. A method for the preparation of a double base propellant grain which comprises the steps of

1. pretreating nitrocellulose by

- a. wetting dry nitrocellulose with methylene chloride,
- b. mixing the wet nitrocellulose into a solution of phenyl isocyanate and methylene chloride,
- c. filtering the mixture to obtain the nitrocellulose, 5
- d. drying the nitrocellulose,
- e. adding water to the nitrocellulose in an amount of about 30 parts water to 70 parts nitrocellulose,
- f. stirring a ballistic modifier with the water wetted nitrocellulose to form a mixture in which the modifier is well dispersed,
- g. drying the mixture;
2. stirring the pretreated nitrocellulose and modifier

15

20

25

30

35

40

45

50

55

60

65

- mixture in a solution of methylene chloride and a casting solvent consisting essentially of an explosive plasticizer, a non-explosive plasticizer and a stabilizer until a slurry is formed,
3. removing methylene chloride from the slurry as stirring continues and as nitrocellulose goes into solution,
  4. adding tolylene diisocyanate to the slurry,
  5. transferring the slurry under reduced pressure to a container, and
  6. curing for from 4 to 7 days at about 50°C.
- \* \* \* \* \*